

## UNITED STATES PATENT OFFICE

2,410,376

## BENEFICIATION OF IRON ORES

Robert Ben Booth, Springdale, and Earl Conrad Herkenhoff, Stamford, Conn., assignors to American Cyanamid Company, New York, N. Y., a corporation of Maine

No Drawing. Application April 5, 1943,  
Serial No. 481,906

8 Claims. (Cl. 209—166)

1

This invention relates to the beneficiation of iron ores by froth flotation processes.

Low grade iron ores have presented a very serious beneficiation problem because the unit value of iron concentrates is not high and flotation procedures in the past have not given commercially useful results. Iron ores containing hematite, magnetite, or similar iron minerals can be subjected to froth flotation in the presence of the typical fatty acid collectors used with oxide ores, but, while some beneficiation takes place, the grade obtained and recovery are not sufficiently high to make the process commercially feasible.

It has been proposed to float oxide ores with water-insoluble reaction products of sulfuric acid and petroleum hydrocarbons from lubricating oil stock obtained as a waste product from the refining lubricating oil stock with strong sulfuric acid, oleum, chlorosulfonic or other sulfonating agents and referred to in the trade as mahogany soaps. These reagents give somewhat better results than fatty acids, but the results are not commercial, particularly when iron ores are treated.

According to the present invention iron ore pulps are treated with an inorganic acid such as sulfuric acid, phosphoric acid and the like, and the acid-treated pulp can be floated with mahogany soaps, used alone, or dispersed in petroleum hydrocarbons, alcohols, or other oily solvents, to give high grades and good recoveries which permit transforming rejected tailings, waste products from washers, and other low grade ores into commercially acceptable concentrates. An outstanding advantage of the concentrates obtained is their generally granular nature which permits easy dewatering, so that concentrates can be shipped to central locations for sintering. The process is also advantageous in that the reagents used are cheap and in normal times readily obtainable in large quantities.

The mechanism of the present invention is not completely known, and it is not desired to limit it to any particular theory of operation. Within wide limits the nature of the acidic anion does not appear to play a great role. Almost any reasonably well dissociated inorganic acid can be used. In fact, it is not necessary to add a free acid. Certain acid salts such as sodium or potassium bisulfate and sodium chlorosulfonate work as well as sulfuric acid. There is some difference in the action of different acids. This leads us to believe that probably one factor of the present invention is the action of the acid on the particles of iron ore. It is possible that another factor may be action on stained gangue such as iron-stained quartz.

It is an advantage of the present invention that the amount of inorganic acid to be used is not critical. This does not mean that the acids

2

may be used in unlimited quantities. With every acid and every ore the effect generally increases at first with the addition of more acid, reaches a maximum, and then may decline when more acid is used. In general, with sulfuric acid, amounts of acid from 1½ to 5 lbs. per ton of flotation feed constitute the range of best operation, with an optimum depending on the ore and other conditions of about 2½ to 3 lbs. per ton. These figures apply to processes in which the pulp is conditioned at high solids. Where conditioning at low solids is employed, such as for example, at flotation pulp density, acceptable results can be obtained, but the amount of acid required is greatly increased, ranging from 5 to 10 lbs. per ton of feed. A commercially acceptable product is obtained, but, because of the better results and smaller reagent consumption, it is preferred to condition at high solids, although the invention is not limited thereto.

The tremendous improvement obtained by means of the present invention is all the more surprising because oxide ore flotation in the presence of anionic collectors such as fatty acids frequently proceeds best in a neutral or slightly alkaline circuit. In fact, the addition of any considerable amounts of sulfuric acid with a fatty acid collector will kill the float altogether. Undoubtedly the acid operates in a different manner with the mahogany soaps. The action does not appear to be one due solely to pH of the circuit, although this may be a contributing factor, because when ore pulp is treated with an acid such as sulfuric acid and then floated in a circuit in which the pH is raised by the addition of an alkali, such as sodium carbonate, the improved results of the present invention are still retained. This is an added reason for believing that at least one factor in the process is some surface effect of the acid on the ore particles.

Water-insoluble reaction products of sulfuric acid and petroleum hydrocarbons from lubricating oil stock vary quite widely with different crude oils and different refining procedures. The compositions are somewhat indefinite and are ordinarily considered to be mixtures containing both sulfonate and sulfate esters. We have found that practically all of these products can be used in the present invention, although there is some difference in effectiveness between mahogany soaps of different petroleum companies. When no acid is used in treating the pulp, there is a very wide difference between mahogany soaps of different origins. It is a surprising effect of the present invention, however, that the acid treatment of the ore to a very great extent adjusts differences between mahogany soaps of different origins. They all give improved results with acid and the difference between various ones is definitely lessened. This curiously different

behaviour with and without acid of various mahogany soaps is an additional reason for believing that one factor of the present invention is a surface alteration of the iron ore and possibly of the gangue. It seems reasonable to believe that the acid treatment may so alter the surface of iron mineral particles that good adherence is obtained with almost any mahogany sulfonate.

It is necessary to coat the mineral particles with the active mahogany soap. This makes it necessary to use some precautions in mixing the promoter with the ore. We have found that it is desirable to have the active ingredients in solution or dispersion in organic solvents. Commercial mahogany soaps are sold as an oil solution or dispersion of the sulfuric acid reaction products and, therefore, are already dispersed in a hydrocarbon solvent. These commercial products may be mixed with the ores directly or they may be further diluted with other organic solvents. The nature of the solvent does not appear to be critical. Excellent results are obtained with hydrocarbon solvents, such as petroleum hydrocarbons which are naturally present in the commercial mahogany soaps, the latter being normally sold in the form of a solution in petroleum hydrocarbons. Glyceride oils, of which cocoanut oil is a typical example, also give good results and it is possible to get good feeding with solutions in various alcohols and other organic materials. This leads us to believe that the main, if not only, function of the solvent is to effect more uniform distribution in the ore pulp, but it may also have other effects, because when it is attempted to feed the active constituents of the mahogany soaps in the form of hot water dispersions the results are not as good. Therefore, it is preferred to introduce the collector in solution in an organic solvent without limiting the invention broadly to this preferred modification.

The question of froth is present as in any froth flotation process, and various mahogany soaps show different frothing powers. Where adequate frothing can be obtained they may be used alone. However, in many cases it is desirable to use one or more frothers, for which the standard types of frothers such as pine oil, cresylic acid, mixtures of higher paraffin alcohols from 7 to 10 carbon atoms and synthetic frothers prepared from mixtures of these higher alcohols with hydrocarbons, may be used. We have also found that water-soluble reaction products of sulfuric acid with petroleum hydrocarbons from lubricating oil stock, the so-called green acids, may also be used as frothers and also show some promoting effect. When used alone with acid treatment, fair results are obtained, but not as good as with the mahogany soaps or acids of the present invention.

The technique of froth flotation is not materially changed by the use of the present invention, and this is an advantage because the operator does not have to learn new techniques, and standard flow-sheets and equipment may be used in most cases. Examples of typical flotation procedures are the use of the process of the present invention in rougher floats, cleaner floats, and the like.

It is also possible to utilize the principles of the present invention in a so-called double-flotation process in which a rougher float is effected with the mahogany soaps or acids on acid treated pulp, adjusting conditions for maximum recovery at some slight sacrifice of grade. The concentrate is then treated with chemicals or agents to remove the collector from the surface of the particles. Typical of such agents are que-

bracho and other dispersing agents. The concentrate with collector removed is then subjected to a cleaning operation using a cationic flotation reagent to float out silica or siliceous gangue. This double float presents a more expensive procedure, but with some highly refractory ores it is an economically attractive procedure.

It is an advantage of the present invention that it may be used in such various manners so as to obtain the best results economically with various ores, taking into consideration the nature of the ore and the economic factors at the mines, such as availability of fuel, shipping costs and the like. In every case the present invention will be used to obtain the best economic results with any particular ore, and the wide latitude given to the ore dressing engineer by the non-critical character of the present invention is of real advantage in permitting optimum results with a wide variety of iron ores.

The problem of slime is not greatly different in the process of the present invention than in the general run of flotation processes. Here, as elsewhere, slime is never desirable. However, it is an advantage of the present invention that it is not peculiarly critical as far as slime is concerned and it is possible to operate with undeslimed ore or, which is more important, with ore which has been only partially deslimed, thus permitting more economical desliming procedures. The effect of slime is normal and manifests itself primarily in added consumption of reagent. As the reagents are fairly cheap it is sometimes desirable to use relatively economical desliming procedures which do not remove the slime completely and such procedures are permissible by reason of the relative lack of sensitivity of the present process to the presence of small amounts of slime. More involved desliming procedures, such as those employing a polishing or scrubbing of the ore particle followed by desliming, are not normally necessary although they may be used and do effect some economy of reagent. The extent to which the desliming is to be effected is largely one of economic compromise and the degree of desliming to produce optimum results with minimum costs will be determined in the case of each ore.

As has been pointed out above, the nature of the acid to be used in treating the ore is not critical. For most practical purposes sulfuric acid is preferred because of its cheapness. It is also one of the best acids. Other acids such as sulfurous acid, phosphoric acid and the like may also be used and in some cases, where waste gases containing  $SO_2$  are available, they constitute a very cheap source of acid usable in the present invention. Within wide limits the purity of the acid does not seem to play any decisive result in the present invention, which permits the use of lower purity acids which are sometimes available at considerably reduced prices and the possibility of using cheap material in the present invention constitutes a further economic advantage.

It is an advantage of the present invention that the addition of acid may take place at various points in the flotation procedure. Thus it may be added in the conditioner and in many cases this is preferable, or it may be used in desliming, or added directly to the flotation circuit. Obviously, of course, the acid may be added in portions at various points in the flotation operation. The fact that the acid addition is not critical permits a great deal of flexibility in setting up a flow sheet for any given iron ore.

The present invention will be described in

greater detail in conjunction with the following specific examples, which are typical of the invention, and which have been chosen to illustrate certain of the ranges within which the invention gives good results. The parts are by weight.

*Example 1*

Minnesota iron ore having an iron content of about 30.5% Fe was deslimed and divided into a large number of portions. Some of these were 10 conditioned at 22% solids with mahogany soaps from various sources and floated in a Fagergren flotation machine. Further tests were made in which the pulp temperature was raised to 50° C. and the mahogany soap fed directly to the flotation cell, these tests being made with and without additional sulfuric acid. Finally further amounts of the ore were treated by conditioning with the promoters and 5 lbs. per ton of sulfuric acid added to the flotation machine. In all tests the mahogany soaps were diluted with 10% secondary butanol. The metallurgical results appear in the following table which is divided into three sections, the first section being the various mahogany soaps, the second, tests at higher temperature, 15 50° C., with and without sulfuric acid, and the third, tests made with 5 lbs. per ton of sulfuric acid at normal temperature.

out above, better results are obtained by conditioning the pulp with promoter at high solids. The significance of the results in Section 3 in the table as compared to Section 1 is, therefore, primarily comparative.

It was attempted to use the various mahogany soaps by feeding them as a 1½% dispersion in hot water directly to the flotation pulp. The use of hot dispersions has been recommended in the past in connection with the use of mahogany soaps as collectors for ores other than iron ores. The results of these tests are not tabulated as in general no flotation took place. The reason for the peculiar behavior of mahogany soaps with iron ore when contrasted with their action on other oxide ores has not been determined, but is probably a surface phenomenon.

The amount of acid present in the treated ore 20 pulp is sufficient to react with the major portion or all of the mahogany soaps to transform them partly or wholly into the corresponding free sulfonic acids. It is possible to use the free sulfonic acids themselves and the results are substantially the same, but it is preferred to use the mahogany soaps, since they are not corrosive and do not present difficulties in shipping or handling.

| Source                                                                                     | Name                        | Lbs./ton | Concentrate        |             |       | Tailing<br>per cent<br>Fe assay |  |
|--------------------------------------------------------------------------------------------|-----------------------------|----------|--------------------|-------------|-------|---------------------------------|--|
|                                                                                            |                             |          | Per cent<br>weight | Per cent Fe |       |                                 |  |
|                                                                                            |                             |          |                    | Assay       | Dist. |                                 |  |
| <i>Section 1</i>                                                                           |                             |          |                    |             |       |                                 |  |
| Standard Oil Company of California                                                         | Calol                       | 2.27     | 31.28              | 44.40       | 46.02 | 23.70                           |  |
| Sonneborn Sons, Inc.                                                                       | Petronate                   | 2.27     | 37.57              | 48.90       | 59.97 | 19.16                           |  |
| Atlantic Refining Co.                                                                      | Ultranate #2                | 2.33     | 31.52              | 49.10       | 50.97 | 21.74                           |  |
| Stanco Distrib., Inc.                                                                      | SP-312                      | 2.40     | 20.01              | 51.90       | 35.64 | 24.95                           |  |
| Do.                                                                                        | SP-302                      | 2.66     | 28.62              | 44.49       | 42.59 | 24.05                           |  |
| Do.                                                                                        | SP-1                        | 2.40     | 43.20              | 46.09       | 65.77 | 18.24                           |  |
| 1:1 mixture of Calol and SP-1                                                              |                             | 2.20     | 32.55              | 44.09       | 47.51 | 23.51                           |  |
| 1 part of above mixture with 1 part of green acids (Sonneborn Sons, Inc.) (water soluble). |                             | 4.40     | 32.93              | 47.98       | 50.28 | 23.30                           |  |
| Sonneborn Sons                                                                             | O-Emulsifier                | 2.67     | 2.87               |             |       |                                 |  |
| Atlantic Refining Co.                                                                      | Ultranate #1                | 2.50     | 11.31              | 48.23       | 18.07 | 27.89                           |  |
| Do.                                                                                        | Ultranate #3                | 2.07     | (2)                |             |       |                                 |  |
| Penna. Oil Prod. Refn'g Co.                                                                | Eldrol                      | 2.13     | 0.92               |             |       |                                 |  |
| Sherwood Refining Co.                                                                      | Reagent 407                 | 2.00     | 0.83               |             |       |                                 |  |
| Shell Oil Co.                                                                              | Crude naphtha sulfonic soap | 1.80     | (2)                |             |       |                                 |  |
| <i>Section 2</i>                                                                           |                             |          |                    |             |       |                                 |  |
| 1:1 mixture of Calol and SP-1                                                              |                             | 2.20     | 7.03               | 46.04       | 10.60 | 29.35                           |  |
| Do. <sup>1</sup>                                                                           |                             | 2.20     | 31.34              | 44.34       | 46.14 | 23.63                           |  |
| Shell Oil Co.                                                                              | Crude naphtha sulfonic soap | 1.80     | 1.42               |             |       |                                 |  |
| Do. <sup>1</sup>                                                                           | do                          | 1.80     | 6.77               | 57.18       | 12.78 | 28.33                           |  |
| <i>Section 3</i>                                                                           |                             |          |                    |             |       |                                 |  |
| Standard Oil Co. of California                                                             | Calol                       | 2.27     | 51.39              | 34.47       | 58.53 | 25.82                           |  |
| Sonneborn Sons                                                                             | Petronate                   | 2.27     | 36.15              | 48.84       | 58.51 | 19.61                           |  |
| 1:1 mixture of Calol and SP-1                                                              |                             | 2.20     | 53.98              | 39.74       | 71.17 | 18.88                           |  |
| Atlantic Refining Co.                                                                      | Ultranate #3                | 2.30     | 55.89              | 40.19       | 74.12 | 17.78                           |  |
| Sonneborn Sons                                                                             | O-Emulsifier                | 2.67     | 38.23              | 52.98       | 68.93 | 15.71                           |  |
| Atlantic Refining Co.                                                                      | Ultranate #1                | 2.50     | 42.34              | 43.97       | 61.77 | 19.98                           |  |
| Penna. Oil Prod. Refn'g Co.                                                                | Eldrol                      | 2.13     | 28.38              | 56.03       | 51.90 | 20.58                           |  |

<sup>1</sup> 2½ lbs. per ton of sulfuric acid added to the flotation.

<sup>2</sup> No promotion.

It will be noted that mahogany soaps or petroleum sulfonates vary considerably in their promoting power. Some show no promotion at all and others, such as, for example, Petronate and SP-1 show considerable promotion, although not sufficient to produce a commercial result. Section 2 shows that high temperature, which has been recommended, produces poorer results and when sulfuric acid is added the results, although not good, are enormously improved. It will also be noted that in Section 3 practically all of the mahogany soaps give good results with 5 lbs. of sulfuric acid. The results in Section 3 are not under the optimum conditions for, as has been pointed

65 A further portion of the Minnesota iron ore used in Example 1 was deslimed and conditioned at high solids (about 67%) with 2 lbs. per ton of Ultranate No. 3, diluted to 22% solids and floated in a Fagergren flotation machine. In the first four tests the sulfonate was prepared as a 12% dispersion in hot water, boiled gently for 10 minutes and then fed to the conditioner, and in the next two tests the sulfonate was fed directly to the conditioner, in the next test in the form of a dispersion in hot 3% sulfuric acid, and in the last test as a dispersion in cold 3% sulfuric acid. In 70 some of the tests sulfuric acid was added and in 75

*Example 2*

others fuel oil. The metallurgical results appear in the following table.

| Sulphonate used, lbs./ton | Lbs./ton                       |          | Concentrate  |             |       | Tailing           |     |
|---------------------------|--------------------------------|----------|--------------|-------------|-------|-------------------|-----|
|                           | H <sub>2</sub> SO <sub>4</sub> | Fuel oil | Per cent wt. | Per cent Fe |       | Per cent Fe assay | pH  |
|                           |                                |          |              | Assay       | Dist. |                   |     |
| 2.0                       | None                           | None     | 1.04         | 60.53       | 84.42 | 8.53              | 7.0 |
| 2.0                       | 2.5                            | None     | 43.30        |             |       |                   | 2.5 |
| 2.0                       | None                           | 2.62     | Nil          |             |       |                   | 7.0 |
| 2.0                       | 2.5                            | 2.67     | 45.09        | 58.69       | 86.05 | 7.80              | 2.5 |
| 2.0                       | None                           | None     | Nil          |             |       |                   | 7.0 |
| 2.0                       | 2.5                            | None     | 42.72        | 59.32       | 82.14 | 9.62              | 2.5 |
| 2.0                       | 2.5                            | None     | 46.34        | 58.46       | 87.91 | 6.94              | 2.5 |
| 2.0                       | 2.5                            | None     | 50.63        | 55.64       | 92.14 | 4.87              | 2.5 |

It will be noted that when no acid was present no flotation resulted. The addition of acid produced an excellent recovery of a material having a commercially acceptable grade. This is quite remarkable as the concentrate is a rougher concentrate only, without any cleaning. The addition of fuel oil alone did not bring about any improvement, but gave good results when associated with sulfuric acid. It will be noted that excellent results were obtained in the last three tests regardless of whether the sulfonate and acid were fed directly or the sulfonate dispersed in the acid.

#### Example 3

A low grade Minnesota iron ore, having about 14.5% Fe chiefly as hematite with a quartz gangue, was deslimed, conditioned at high solids (67%) with 2 lbs. per ton of Petronate, diluted to flotation density and floated in a Fagergren flotation machine. In the first two tests the sulfonate was fed directly to the conditioner, in the third test the sulfonate was prepared as a 12% dispersion in hot water, and in the last test this 12% dispersion was boiled gently for 10 minutes prior to feeding. The metallurgical results appear in the following table.

| Sulphonate used, lbs./ton | Lbs./ton H <sub>2</sub> SO <sub>4</sub> | Concentrate  |             |       | Tailing           |     |
|---------------------------|-----------------------------------------|--------------|-------------|-------|-------------------|-----|
|                           |                                         | Per cent wt. | Per cent Fe |       | Per cent Fe assay | pH  |
|                           |                                         |              | Assay       | Dist. |                   |     |
| 2.0                       | None                                    | 15.10        | 52.50       | 61.48 | 5.85              | 6.9 |
| 2.0                       | 2.5                                     | 20.33        | 52.86       | 83.43 | 2.68              | 2.3 |
| 2.0                       | 2.5                                     | 23.40        | 52.25       | 92.90 | 1.22              | 2.5 |
| 2.0                       | 2.5                                     | 24.43        | 50.43       | 96.40 | 0.61              | 2.5 |

It will be noted that Petronate gives considerable beneficiation even without the presence of sulfuric acid, but the acid greatly increases the recovery. Under the best conditions with good dispersion the recovery is increased by about 50%. While the grade is slightly below commercial standard, which usually requires about 58% Fe, it is sufficiently high so that commercial results may be obtained by cleaning.

#### Example 4

The ore of Example 1 was used in a series of tests in which it was conditioned at high solids (67%) with various mahogany soaps, then diluted and floated using a rougher float and cleaner float. The amount of sulfuric acid was kept constant at 2½ lbs. per ton. The metallurgical results appear in the following table in which the first line for the first 5 mahogany soaps represents rougher floats and the second line cleaner floats. In the case of the last reagent, rougher

flotation alone is given, as the results of rougher flotation are commercial.

| 5  | Sulphonate used <sup>1</sup>  |          | Concentrate  |             |       | Tailing per cent Fe assay |  |
|----|-------------------------------|----------|--------------|-------------|-------|---------------------------|--|
|    | Name                          | Lbs./ton | Per cent wt. | Per cent Fe |       |                           |  |
|    |                               |          |              | Assay       | Dist. |                           |  |
| 10 | Petronate                     | 3.60     | 56.46        | 46.35       | 84.70 | 10.86                     |  |
|    | Ultramate #2                  | 3.49     | 56.82        | 49.61       | 91.93 | 5.73                      |  |
|    | SP-312                        | 3.25     | 48.30        | 53.81       | 84.94 | 8.91                      |  |
| 15 | Ultramate #1                  | 3.84     | 55.07        | 47.14       | 84.33 | 10.74                     |  |
|    | Ultramate #3                  | 2.20     | 54.93        | 51.76       | 93.44 | 4.43                      |  |
|    | 1:1 mixture of Calol and SP-1 | 2.20     | 39.63        | 58.68       | 76.71 | 11.69                     |  |

<sup>1</sup> All sulfonates diluted with 10% secondary butanol.

#### Example 5

The effects of various acid concentrations were tested using the deslimed ore of Example 1 conditioned at high solids with 2.2 lbs. per ton of an equal mixture of Calol and SP-1 diluted with 10% secondary butanol, followed by dilution to flotation density and flotation in a Fagergren flotation machine. The metallurgical results are as follows:

| 30 | H <sub>2</sub> SO <sub>4</sub> , lbs./ton | Rougher concentrate |             |       | Tailing           |     |
|----|-------------------------------------------|---------------------|-------------|-------|-------------------|-----|
|    |                                           | Percent wt.         | Per cent Fe |       | Per cent Fe assay | pH  |
|    |                                           |                     | Assay       | Dist. |                   |     |
| 35 | None                                      | 9.23                | 43.80       | 13.20 | 29.28             | 7.0 |
|    | 0.50                                      | 46.04               | 54.05       | 81.39 | 10.54             | 5.7 |
|    | 1.50                                      | 42.95               | 58.32       | 82.10 | 9.57              | 3.1 |
| 40 | 2.50                                      | 39.63               | 58.68       | 76.71 | 11.69             | 2.7 |

It will be noted that, as the amount of sulfuric acid increased, the results improved up to about 1½ lbs. per ton, reaching a maximum at about this point, with some loss in recovery when 2½ lbs. per ton of sulfuric acid was reached. With this reagent combination a pH of about 3 gives best results. It should be noted that in a single roughing operation, high recovery of a commercial grade of concentrate was obtained without any cleaning.

#### Example 6

The effect of conditioning time was studied, using the deslimed ore of Example 1, conditioning being effected at 67% solids, followed by dilution to flotation density and flotation in a Fagergren flotation machine. In each case the reagent was an equal mixture of Calol and SP-1 in the amount of 2.2 lbs. per ton associated with 2½ lbs. per ton of sulfuric acid. The sulfonate mixture was diluted with 10% secondary butanol. The metallurgical results appear in the following table.

| 65 | Rougher concentrate |             |       | Tailing assay, per cent Fe | Time of conditioning |  |  |
|----|---------------------|-------------|-------|----------------------------|----------------------|--|--|
|    | Per cent wt.        | Per cent Fe |       |                            |                      |  |  |
|    |                     | Assay       | Dist. |                            |                      |  |  |
| 70 | 39.63               | 58.68       | 76.71 | 11.69                      | Minutes              |  |  |
|    | 41.82               | 59.29       | 81.77 | 9.50                       | 2                    |  |  |
|    | 22.22               | 50.68       | 43.31 | 22.31                      | 4                    |  |  |
|    |                     |             |       |                            | 6                    |  |  |

It will be noted that as the time of conditioning increases so does the recovery, but excessive conditioning brings about a drop. The reason for this phenomenon is not known. However, the change is not sudden and the conditioning time is, therefore, not critical.

*Example 7*

This test was made to show the results obtainable with various types of iron ore. In every case the ores were deslimed, conditioned at high solids with an equal mixture of Calol and SP-1 (diluted with 10% secondary butanol) and optimum amounts of sulfuric acid. The conditioned pulp was then diluted to flotation density and floated in a Fagergren flotation machine. The results appear in the following table; the first, fourth and fifth and last ores were cleaned once; the second and third ores cleaned twice; and the sixth and seventh ores a rougher concentrate only taken.

| Sulfonate used, lbs./ton | H <sub>2</sub> SO <sub>4</sub> , lbs./ton | Ore        |                              | Feed assay, per cent Fe | Concentrate  |             | Final tailing |                   |     |
|--------------------------|-------------------------------------------|------------|------------------------------|-------------------------|--------------|-------------|---------------|-------------------|-----|
|                          |                                           | Source     | Principal minerals           |                         | Per cent wt. | Per cent Fe |               | Per cent Fe assay |     |
|                          |                                           |            |                              |                         |              | Assay       | Dist.         |                   |     |
| 3.30                     | 3.0                                       | Minnesota  | Hematite and quartz          | 14.06                   | 20.14        | 55.39       | 79.35         | 3.17              | 2.6 |
| 7.70                     | 2.5                                       | New Jersey | Magnetite and quartz         | 50.50                   | 62.80        | 57.34       | 72.45         | 41.11             | 6.0 |
| 6.60                     | 3.8                                       | Canada     | Hematite and quartz          | 27.06                   | 46.51        | 49.17       | 84.52         | 3.66              | 2.8 |
| 3.30                     | 2.5                                       | Minnesota  | do                           | 12.74                   | 19.48        | 58.34       | 92.01         | 0.85              | 2.3 |
| 2.93                     | 3.3                                       | do         | do                           | 19.55                   | 28.72        | 58.22       | 85.52         | 1.71              | 2.4 |
| 2.20                     | 5.0                                       | New Jersey | Magnetite and quartz         | 65.17                   | 78.99        | 70.89       | 85.92         | 43.66             | 2.1 |
| 2.20                     | 3.5                                       | Minnesota  | Magnetite and iron silicates | 49.52                   | 64.77        | 58.07       | 75.95         | 38.40             | 2.6 |
| 2.20                     | 2.5                                       | do         | Hematite and quartz          | 22.03                   | 37.09        | 53.96       | 90.83         | 2.49              | --- |

It will be noted that commercial grades are obtained with all ores except the low grade Minnesota ore which was cleaned only once and the Canadian ore which proved very refractory but which showed marked beneficiation. These results are typical since, as has been pointed out above, while the present invention is applicable generally to all iron ores, the results will vary from ore to ore.

*Example 8*

A number of pure minerals were floated to show the response to various amounts of sulfuric acid. The results appear in the following table.

| Mineral                             | H <sub>2</sub> SO <sub>4</sub> , lbs./ton | Petronate, lbs./ton | pH  | Weight, grams |       |       | Per cent floated |
|-------------------------------------|-------------------------------------------|---------------------|-----|---------------|-------|-------|------------------|
|                                     |                                           |                     |     | Feed          | Float | Tail. |                  |
| Hematite                            | None                                      | 5.0                 | 6.4 | 29.9          | 1.6   | 28.3  | 5.4              |
| Do                                  | 2.0                                       | 5.0                 | 5.3 | 29.3          | 17.2  | 12.1  | 58.7             |
| Do                                  | 4.0                                       | 5.0                 | 3.7 | 30.5          | 20.4  | 10.1  | 66.9             |
| Do                                  | 8.0                                       | 5.0                 | 2.7 | 30.6          | 26.4  | 4.2   | 86.3             |
| Do                                  | 16.0                                      | 5.0                 | 2.3 | 30.4          | 26.4  | 4.0   | 86.9             |
| Martite <sup>1</sup>                | None                                      | 5.0                 | 7.9 | 30.2          | 8.1   | 22.1  | 26.8             |
| Do                                  | 8.0                                       | 5.0                 | 2.5 | 30.3          | 29.8  | 0.5   | 98.3             |
| Limonite                            | None                                      | 5.0                 | 7.9 | 31.3          | 15.7  | 15.6  | 50.2             |
| Do                                  | 8.0                                       | 5.0                 | 2.5 | 32.6          | 31.3  | 1.3   | 96.0             |
| Goethite                            | None                                      | 1.0                 | 6.2 | 30.5          | 10.3  | 20.2  | 33.8             |
| Do                                  | 8.0                                       | 1.0                 | 2.2 | 29.9          | 24.2  | 5.7   | 81.0             |
| Magnetite <sup>1</sup>              | None                                      | 5.0                 | 6.9 | 30.5          | 9.4   | 21.1  | 30.8             |
| Do                                  | 8.0                                       | 5.0                 | 2.3 | 31.1          | 29.5  | 1.6   | 94.9             |
| Titaniferous magnetite <sup>1</sup> | None                                      | 5.0                 | 6.7 | 29.6          | 9.3   | 20.3  | 31.4             |
| Do                                  | 8.0                                       | 5.0                 | 2.3 | 29.8          | 28.9  | 0.9   | 97.0             |
| Siderite                            | None                                      | 1.0                 | 6.4 | 30.5          | 6.6   | 23.9  | 21.6             |
| Do                                  | 2.0                                       | 1.0                 | 3.3 | 30.8          | 30.0  | 0.8   | 97.5             |
| Ilmenite                            | None                                      | 1.0                 | 7.4 | 30.3          | 20.0  | 10.3  | 66.0             |
| Do                                  | 4.0                                       | 1.0                 | 2.4 | 30.3          | 30.1  | 0.2   | 99.3             |

<sup>1</sup> In absence of acid, froth was excessive, causing much mechanical overflow into the float products.

*Example 9*

The effect of temperature was studied, using another low grade Minnesota ore. The ore, which

contained about 14.3% Fe with a quartz gangue, was deslimed, conditioned at 65% solids with 2.2 lbs. per ton of an equal mixture of Calol and SP-1 (diluted with 10% secondary butanol), together with 2.5 lbs. per ton of sulfuric acid. The conditioned pulp was then diluted to flotation density and floated in a Fagergren flotation machine. The metallurgical results appear in the following table.

| Assay | Dist. | Tailing           |     | Temp. of pulp |
|-------|-------|-------------------|-----|---------------|
|       |       | Per cent Fe assay | pH  |               |
| 43.24 | 87.19 | 2.44              | 2.4 | 5             |
| 43.82 | 91.90 | 1.53              | 2.4 | 12            |
| 39.22 | 89.85 | 2.07              | 2.4 | 30            |
| 42.84 | 77.66 | 4.14              | 2.4 | 60            |

It will be noted that optimum results are ob-

tained below 30° C. and there is a marked loss in recovery at 60° C. The excellent results at 5° C. are quite significant as flotation operations in Minnesota and other northern iron districts must frequently be conducted at comparatively low temperatures so that the characteristic of the present invention of giving good results at low temperatures is of great practical importance.

*Example 10*

The effect of various pulp densities in conditioning was tested using the deslimed ore of Example 1. Conditioning with 2.2 lbs. per ton of an equal mixture of Calol and SP-1 (diluted

with 10% secondary butanol) and 2.5 lbs. per ton of sulfuric acid was effected at various pulp densities, followed by dilution to 22% solids and flota-

## 11

tion in a Fagergren flotation machine. The metallurgical results appear in the following table.

| Concentrate,<br>per cent Fe |       | Tailing              |       | Pulp density<br>per cent<br>solids in<br>conditioning |
|-----------------------------|-------|----------------------|-------|-------------------------------------------------------|
| Assay                       | Dist. | Per cent<br>Fe assay | pH    |                                                       |
| 57.86                       | 82.88 | 9.62                 | 2.3   | 67                                                    |
| 49.94                       | 82.95 | 11.21                | ----- | 52                                                    |
| 43.12                       | 91.35 | 7.19                 | ----- | 36                                                    |
| 32.57                       | 88.55 | 19.64                | 2.3   | 22                                                    |

The above tests show that optimum grade is obtained with high solids conditioning. Conditioning at lower solids, while permitting excellent recoveries, decreases very markedly the degree of concentration.

## Example 11

The effect of flotation pulp density was studied, using the ore of Example 10, conditioning being effected at 67% solids with the same amount of the same reagent and acid, followed by flotation in a Fagergren flotation machine at various pulp densities. The metallurgical results appear in the following table.

| Concentrate             |       | Tailing              |       | Pulp density<br>per cent<br>solids in<br>flotation |
|-------------------------|-------|----------------------|-------|----------------------------------------------------|
| Per cent<br>Fe<br>assay | Dist. | Per cent<br>Fe assay | pH    |                                                    |
| 60.29                   | 86.32 | 7.31                 | 2.4   | 11                                                 |
| 57.86                   | 82.88 | 9.62                 | ----- | 22                                                 |
| 53.84                   | 89.15 | 6.94                 | ----- | 33                                                 |

The variation of flotation pulp density causes a considerable change in grade, the best results being at the very low density of 11%. At this density, however, the capacity of the machine is decreased and the particular density to be chosen will be the result of an economic compromise between output and grade.

## Example 12

The effect of slime was determined, using a low grade Minnesota iron ore. This ore was divided into three portions, the first of which was deslimed thoroughly, the second was not deslimed at all, and the third was partially deslimed. Conditioning was effected at high solids with the secondary butanol mixture of Calol and SP-1 and sulfuric acid, the optimum amounts of reagent and acid being used in each case. The metallurgical results appear in the following table.

| Product                           | Assay          |                    | Consumption,<br>lbs./ton |                |                                |
|-----------------------------------|----------------|--------------------|--------------------------|----------------|--------------------------------|
|                                   | Per cent<br>Fe | Per cent<br>insol. |                          | Sulfon-<br>ate | H <sub>2</sub> SO <sub>4</sub> |
| Substantially complete desliming: |                |                    |                          |                |                                |
| Calc. head                        | 14.53          | -----              | 100.00                   |                |                                |
| Slime                             | 40.92          | -----              | 17.84                    |                |                                |
| Clean. conc.                      | 60.17          | 7.00               | 75.60                    | 2.20           | 2.50                           |
| Clean. tail                       | 11.57          | 81.70              | 2.32                     |                |                                |
| Rough. tail                       | 0.85           | -----              | 4.24                     |                |                                |
| Rough. conc.                      | 53.49          | -----              | 77.92                    |                |                                |
| No desliming:                     |                |                    |                          |                |                                |
| Calc. head                        | 14.55          | -----              | 100.00                   | Conc. #1       |                                |
| Conc. No. 1                       | 41.53          | -----              | 28.38                    | 4.40           | 5.00                           |
| Clean. conc. No. 2                | 55.05          | 15.00              | 42.16                    | Conc. #2       |                                |
| Clean. tail                       | 15.47          | 75.20              | 10.34                    | 2.20           |                                |
| Rough. tail                       | 4.02           | -----              | 19.12                    |                |                                |
| Rough. conc. No. 2                | 36.61          | -----              | 52.50                    |                |                                |
| Partial desliming:                |                |                    |                          |                |                                |
| Calc. head                        | 14.22          | -----              | 100.00                   |                |                                |
| Slime                             | 35.93          | -----              | 15.54                    |                |                                |
| Rough. conc.                      | 56.52          | 12.70              | 62.36                    | 2.20           | 2.50                           |
| Tailing                           | 4.02           | -----              | 22.10                    |                |                                |

## 12

It will be apparent that desliming is helpful, although the presence of slime does not preclude obtaining fair results but at a higher cost for reagents.

5

## Example 13

The effect of various acids was determined by testing with a low grade ore such as that described in Example 12. In every case the ore was conditioned at high solids with 2.2 lbs. per ton of an equal mixture of Calol and SP-1 diluted with 10% secondary butanol. Rougher flotation only was conducted. The metallurgical results are shown in the following table.

15

| Type                              | Lbs./ton | Acid used          |                | Concentrate             |      | Tailing |  |
|-----------------------------------|----------|--------------------|----------------|-------------------------|------|---------|--|
|                                   |          | Per cent<br>weight | Per cent<br>Fe | Assay<br>per cent<br>Fe | pH   |         |  |
|                                   |          | Assay              | Dist.          |                         |      |         |  |
| None—control test                 |          | 13.87              | 52.98          | 58.60                   | 6.03 | 6.8     |  |
| Hydrochloric                      | 2.5      | 24.39              | 46.04          | 91.72                   | 1.34 | 2.7     |  |
| Nitric                            | 2.5      | 26.74              | 44.09          | 92.31                   | 1.34 | 2.7     |  |
| Hydrofluoric—<br>49%              | 3.54     | 22.52              | 51.89          | 91.18                   | 1.46 | 2.8     |  |
| Hydrofluosilicic—<br>16 (27%-30%) | 3.99     | 23.01              | 50.91          | 92.23                   | 1.22 | 2.5     |  |
| Boric                             | 2.5      | 14.17              | 54.20          | 62.45                   | 5.38 | 6.8     |  |
| Perchloric                        | 2.5      | 26.57              | 43.20          | 89.72                   | 1.79 | 2.7     |  |
| Phosphoric                        | 2.5      | 21.12              | 52.69          | 88.74                   | 1.79 | 2.7     |  |
| Sulfurous                         | 2.5      | 19.93              | 55.77          | 90.02                   | 1.54 | 2.3     |  |
| Carbonic                          | (1)      | 25.50              | 43.92          | 89.74                   | 1.72 | 6.1     |  |

30

<sup>1</sup> Saturated.

The acids all show improved recovery, although there is considerable variation. A very weak acid, such as boric acid, is not sufficiently effective for economical operations on a commercial scale. In general, a dissociation constant between 10<sup>-7</sup> and 10<sup>-8</sup> represents the lower limit of utility.

35

## Example 14

Various dispersing agents can be used in the present process prior to desliming. The following tests were made. The ore used was that of Example 1 and the dispersing agents were added prior to desliming. In each case conditioning was effected at high solids with 2.2 lbs. of the secondary butanol mixture of Calol and SP-1 and 2.5 lbs. per ton of sulfuric acid (except in the case of sodium hydroxide, where 3.5 pounds of sulfuric acid per ton were used in order to neutralize the alkalinity). The pulp was diluted to flotation density, and floated in a Fagergren flotation machine with a single cleaning. The following metallurgical results were obtained.

55

| Name                             | Lbs./ton | Additional reagents |                | Concentrate |       | Tailing<br>per cent<br>Fe<br>assay |
|----------------------------------|----------|---------------------|----------------|-------------|-------|------------------------------------|
|                                  |          | Percent<br>wt.      | Per cent<br>Fe | Assay       | Dist. |                                    |
| Sodium silicate                  | 3.00     | 42.56               | 60.25          | 84.35       |       | 5.26                               |
| Sodium diethyl sulfosuccinate    | 0.50     | 37.77               | 61.41          | 68.71       |       | 11.54                              |
| Sodium hydroxide                 | 2.00     | 42.14               | 60.77          | 85.05       |       | 5.13                               |
| Calcium lignin sulfonate (crude) | 2.00     | 39.97               | 61.41          | 81.26       |       | 6.67                               |

60

It will be noted that the use of the dispersing agents does not adversely affect the flotation operation, which is an added advantage of the present invention as it permits the use of agents which aid in desliming.

65

## Example 15

A number of tests were run with the deslimed ore of Example 1 to determine the effects of vary-

70

75

ing amounts of fuel oil and reagents. In every case the deslimed ore was conditioned at high solids with the reagent and 2.5 lbs. per ton of sulfuric acid were used in the conditioning. The first four tests used a constant amount of reagent, 2.2 lbs. per ton of an equal mixture of Calol and SP-1, diluted with 10% secondary butanol, and the second four tests used a constant amount of fuel oil, 1.12 lbs. per ton, and varying amounts of the alcoholic mixture of Calol and SP-1. The metallurgical results are shown in the following table.

| Sulfonate used, lbs./ton     | Lbs./ton      |          | Concentrate     |             |       | Tailing assay, per cent Fe |  |
|------------------------------|---------------|----------|-----------------|-------------|-------|----------------------------|--|
|                              | Sulfuric acid | Fuel oil | Per cent weight | Per cent Fe |       |                            |  |
|                              |               |          |                 | Assay       | Dist. |                            |  |
| 2.20                         | 2.50          | None     | 45.38           | 56.52       | 84.26 | 8.77                       |  |
| 2.20                         | 2.50          | 0.56     | 47.32           | 56.58       | 89.54 | 5.97                       |  |
| 2.20                         | 2.50          | 1.12     | 47.09           | 58.83       | 90.07 | 5.77                       |  |
| 2.20                         | 2.50          | 2.24     | 32.50           | 58.83       | 62.79 | 16.79                      |  |
| 1.65                         | 2.50          | 1.12     | 28.34           | 57.82       | 53.98 | 19.49                      |  |
| 2.20                         | 2.50          | 1.12     | 47.09           | 58.83       | 90.07 | 5.77                       |  |
| 2.75                         | 2.50          | 1.12     | 50.09           | 57.31       | 94.53 | 3.33                       |  |
| 3.30                         | 2.50          | 1.12     | 51.94           | 56.44       | 96.60 | 2.15                       |  |
| After one cleaning operation |               | 48.58    | 59.61           | 95.42       | ----- |                            |  |

It will be noted that there is an optimum amount of fuel oil and an optimum amount of reagent. These amounts will vary somewhat from ore to ore and from reagent to reagent.

#### Example 16

The following tests were made to compare various organic solvents and materials used in combination with mahogany soap. The ore and conditioning procedure was the same as in the preceding example. In each case 2.2 lbs. per ton of an equal mixture of Calol and SP-1, diluted with 10% secondary butanol, and 2.5 lbs. per ton of sulfuric acid were used in the conditioning step, at which time the additional reagent was also introduced. After dilution to flotation density the pulp was floated in a Fagergren flota-

It will be apparent that the present invention is not at all critical with respect to the organic solvent used, commercially acceptable results both from the standpoint of grade and recovery being obtained in each case.

#### Example 17

A further series of tests was made on the ore used in Example 16, but a different petroleum sulfonate, namely Ultramate No. 3, was employed. In each case the reagent consisted of 3 parts of Ultramate No. 3 to 1 part of the organic solvent. The amount of sulfuric acid used was 2.5 lbs. per ton as in the preceding example. A rougher concentrate only was taken. The metallurgical results appear in the following table.

| Organic solvent | Reagent used, lbs./ton | Concentrate  |             | Tailing assay, per cent Fe |      |
|-----------------|------------------------|--------------|-------------|----------------------------|------|
|                 |                        | Per cent wt. | Per cent Fe |                            |      |
|                 |                        |              | Assay       | Dist.                      |      |
| Cocoonut oil    | 2.06                   | 42.28        | 59.54       | 83.31                      | 8.74 |
| Kerosene        | 2.50                   | 46.13        | 59.16       | 89.35                      | 6.04 |
| Ethyl alcohol   | 2.42                   | 46.12        | 58.90       | 90.32                      | 5.40 |

#### Example 18

The use of acid salts instead of acids was illustrated by the following tests in which a deslimed ore similar to that in Example 1 was used, being conditioned at high solids with varying amounts of the secondary butanol mixture of Calol and SP-1 and acid salts. After dilution to flotation density in the first test a roughing float followed by a single cleaning was used and in the second test a rougher concentrate only was taken. The metallurgical results appear in the following table.

| Sulfonate used, lbs./ton | Acid salt              |          | Concentrate  |             | Tailing |                    |
|--------------------------|------------------------|----------|--------------|-------------|---------|--------------------|
|                          | Name                   | Lbs./ton | Per cent wt. | Per cent Fe |         | Assay, per cent Fe |
|                          |                        |          |              | Assay       | Dist.   |                    |
| 4.40                     | Potassium bisulfate    | 10.0     | 44.00        | 60.96       | 88.64   | 4.89               |
| 2.20                     | Sodium chlorosulfonate | 6.0      | 42.78        | 59.28       | 83.12   | 9.00               |

#### Example 19

The double flotation of Minnesota iron ore containing about 29% Fe was carried out by desliming the ore, conditioning with 2.2 lbs. per ton of an equal mixture of Calol and SP-1 (diluted with 10% secondary butanol) and 2.5 lbs. per ton of sulfuric acid. The conditioning took place at 67% solids. The conditioned pulp was then diluted, subjected to flotation, conditioned with additional 1.1 lbs. per ton of the sulfonate mixture and again floated, followed by treatment of the concentrate with quebracho and soda ash and desliming. Cationic flotation with pine oil and 75 laurylamine hydrochloride was then conducted.

Additional reagent

| Name                        | Lbs./ton | Concentrate  |             |       | Tailing assay, per cent Fe |  |
|-----------------------------|----------|--------------|-------------|-------|----------------------------|--|
|                             |          | Per cent wt. | Per cent Fe |       |                            |  |
|                             |          |              | Assay       | Dist. |                            |  |
| Oleic acid                  | 0.75     | 49.81        | 57.82       | 94.12 | 2.69                       |  |
| Tallow                      | 0.75     | 51.10        | 57.05       | 95.09 | 2.44                       |  |
| Naphthenic acid             | 0.68     | 43.39        | 59.36       | 84.30 | 6.79                       |  |
| Cottonseed oil              | 0.70     | 45.09        | 60.25       | 88.42 | 3.72                       |  |
| Toluene                     | 0.50     | 42.49        | 60.25       | 83.35 | 6.15                       |  |
| Crude oil (Calif.)          | 0.68     | 47.53        | 58.97       | 92.65 | 2.31                       |  |
| Lauryl alcohol              | 0.67     | 42.57        | 60.38       | 83.15 | 6.28                       |  |
| Dibutyl phthalate           | 1.00     | 35.41        | 59.87       | 69.61 | 11.15                      |  |
| Cocoonut oil                | 0.74     | 45.72        | 60.90       | 90.15 | 3.85                       |  |
| n-Heptadecene               | 0.83     | 39.26        | 59.23       | 75.77 | 10.26                      |  |
| Chlorinated kerosene        | 0.63     | 45.01        | 59.74       | 87.47 | 3.33                       |  |
| Fuel oil No. 2 <sup>1</sup> | 1.12     | 47.09        | 58.83       | 90.07 | 5.77                       |  |

<sup>1</sup> Rougher flotation only.

The flotation procedure and metallurgical results are tabulated in the following table.

| Operation           | Flotation per cent solids | Quebracho, lbs./ton | Soda ash, lbs./ton | Pine oil, lbs./ton | Laurylamine hydrochloride, lbs./ton |
|---------------------|---------------------------|---------------------|--------------------|--------------------|-------------------------------------|
| Deslime             |                           |                     |                    |                    |                                     |
| Conditioner         | 67                        |                     |                    |                    |                                     |
| Flotation—anionic   | 22                        |                     |                    |                    |                                     |
| Condition the conc. | 13                        | 2.0                 | 2.0                |                    |                                     |
| Deslime             |                           |                     |                    |                    |                                     |
| Flotation—cationic  |                           |                     |                    | 0.108              | 0.35                                |

## RESULTS

| Product         | Per cent wt. | Assay per cent Fe | Dist. per cent Fe |
|-----------------|--------------|-------------------|-------------------|
| Head            | 100.00       | 28.98             | 100.00            |
| Primary slime   | 5.14         | 22.89             | 4.06              |
| Rougher tailing | 39.70        | 2.57              | 3.52              |
| Secondary slime | 4.06         | 15.69             | 2.20              |
| Silica conc.    | 4.45         | 24.18             | 3.71              |
| Iron tailing    | 46.65        | 53.75             | 86.51             |

## Example 20

A deslimed ore such as used in Example 1 was subjected to conditioning at high solids with an equal mixture of Calol and SP-1, diluted with 10% secondary butanol, and various tests were run; first with 2.5 lbs. of sulfuric acid, then with no acid but soda ash in the conditioning, and finally acid treatments followed by neutralization of the acidity with soda ash in the flotation circuit. The various samples of ore were then diluted to flotation density, floated in a Fagergren flotation machine to produce a rougher concentrate and, following the addition of more sulfonate a scavenger concentrate, the scavenger concentrate being intended to be treated as a middling and recycled in the circuit. The metallurgical results appear in the following table in which the scavenger concentrate appears in the second line of each successful test.

| Sulfonate used, lbs./ton | Sulfuric acid, lbs./ton | Soda ash, lbs./ton | Concentrate Per cent Fe  |       | Final tailing      |      |
|--------------------------|-------------------------|--------------------|--------------------------|-------|--------------------|------|
|                          |                         |                    | Assay                    | Dist. | Assay, per cent Fe | pH   |
| 2.20                     | 2.5                     | None               | 58.68                    | 76.71 | —                  | —    |
| 1.10                     | —                       | None               | 39.28                    | 15.06 | 5.12               | 2.6  |
| 2.20                     | —                       | 5.0                | No useful float produced | —     | —                  | 10.0 |
| 2.20                     | 2.5                     | 3.0                | 57.43                    | 79.49 | —                  | —    |
| 1.10                     | —                       | None               | 27.69                    | 13.05 | 5.26               | 6.8  |
| 2.20                     | 2.5                     | 4.0                | 59.10                    | 65.95 | —                  | —    |
| 1.10                     | —                       | None               | 39.49                    | 23.21 | 6.92               | 7.3  |

The results clearly show that, in the absence of acid, soda ash prevents any useful float, whereas if the ore has been treated with acid, a considerable amount of soda ash, up to the amount which results in an almost neutral circuit, does not adversely affect the recovery and grade. When the amount of soda ash is increased still further some falling off in recovery is to be noted, but in this case the grade of the scavenger concentrate is much higher and, therefore, a considerable portion of the iron values would be recoverable therefrom. This results in an overall iron recovery when recycling of the middlings is employed, which is not substantially poorer than with smaller amounts of soda ash. The reason for the curious behaviour of acid-treated ore is not known, but it indicates that the pH of the flotation circuit is not the controlling factor. This is an added advantage of the present inven-

tion because it permits obtaining good results with many iron ores in a flotation circuit which is sub-

stantially neutral, and, therefore, does not present a serious corrosion problem, making it unnecessary to use acid-proof material except in the conditioner which is a type of apparatus more readily acid-proofed than flotation machines. Any of the ordinary alkalies, such as caustic soda or ammonia, may be used. Alkalies which form insoluble compounds, such as lime, do not give quite as good results. Because of its relatively low cost and excellent results, soda ash is normally preferred.

In the examples the invention has been described in connection with the use of a Fagergren flotation machine. This machine gives excellent results in the process of the present invention and is preferred. However, the process of the present invention is in no sense limited to any particular flotation machine and any of the ordinary types of flotation machines may be employed.

All of the oil soluble petroleum sulfonates referred to in the examples under the trade names are typical petroleum sulfonates of the mahogany soap or acid type as commercially obtained from the treatment of petroleum lubricating oil fractions with sulfonating agents, such as sulfuric acid, oleum and the like.

We claim:

1. A method of beneficiating oxidized iron ores by froth flotation of the ore in the form of an aqueous pulp, which comprises conditioning the ore with an inorganic acid substance, the anion of which is a constituent of an inorganic acid having a dissociation constant of at least  $10^{-7}$ , the amount of said acid substance being such that on dilution to froth flotation density and floating, the rougher tailing in the absence of added alkali shows a pH in the range of 2 to 6, and subjecting the aqueous pulp of said treated ore to froth flotation in the presence of a collector for oxidized iron minerals, the major constituent of which is an oil soluble petroleum sulfonate obtained in the refining of petroleum lubricating oils and removing a concentrate relatively rich in iron and a tailing relatively poor in iron.

2. A method of beneficiating oxidized iron ores by froth flotation of the ore in the form of an aqueous pulp, which comprises conditioning the ore with sulfuric acid, the amount of said sulfuric acid being such that on dilution to froth flotation density and floating, the rougher tailing in the absence of added alkali shows a pH in the range of 2 to 6, and subjecting the aqueous pulp of said treated ore to froth flotation in the presence of a collector for oxidized iron minerals, the major constituent of which is an oil soluble petroleum sulfonate obtained in the refining of petroleum lubricating oils and removing a concentrate relatively rich in iron and a tailing relatively poor in iron.

3. A method according to claim 1 in which conditioning is effected at high solids with both collector and acid substance and the thus condi-

tioned pulp is then diluted to flotation density before froth flotation.

4. A method according to claim 2 in which conditioning is effected at high solids with both collector and sulfuric acid and the thus conditioned pulp is then diluted to flotation density before froth flotation.

5. A method according to claim 1 in which the conditioning is with a mixture of petroleum sulfonate and an unsulfonated oil.

6. A method according to claim 2 in which

the conditioning is with a mixture of petroleum sulfonate and an unsulfonated oil.

7. A method according to claim 1 in which the conditioning is at high solids with the acid substance, petroleum sulfonate and unsulfonated oil.

8. A method according to claim 2 in which the conditioning is at high solids with sulfuric acid, petroleum sulfonate and unsulfonated oil.

ROBERT BEN BOOTH.  
EARL CONRAD HERKENHOFF.